

Sept. 19, 1939.

J. O. BETTERTON ET AL

2,173,268

PROCESS FOR RECOVERING TIN

Filed Dec. 2, 1935

*Fig. 1*



*Fig. 2*



INVENTORS  
Jesse O. Betterton  
BY Yurii E. Lebedeff

James H. Kent  
ATTORNEY

## UNITED STATES PATENT OFFICE

2,173,268

## PROCESS FOR RECOVERING TIN

Jesse O. Betterton and Yurii E. Lebedeff,  
Metuchen, N. J., assignors to American Smelt-  
ing and Refining Company, New York, N. Y.,  
a corporation of New Jersey

Application December 2, 1935, Serial No. 52,450

7 Claims. (Cl. 204—17)

This invention relates to the metallurgy of tin and provides an improved electrochemical process for recovering metallic tin from stannic chloride.

5 In treating secondary metals containing tin, such as impure solder and other tin alloys, the tin may be separated by chloridization, e. g. by reaction of the molten alloy with chlorine gas thereby converting the tin to tin tetrachloride, which 10 is volatile at the temperatures employed and is readily recovered by condensation.

By the process of the present invention tin is precipitated from an aqueous stannic chloride electrolyte in a galvanic cell equipped with electrodes of dissimilar materials and is recovered in a form readily amenable to melting down to pig metal.

In accordance with the invention, the electrolyte is placed in a cell equipped with a cathode 20 which is electronegative with respect to tin, e. g., copper or mercury and a soluble anode which is electropositive with respect to tin, e. g., zinc or aluminum. Suitable electrical connection between anode and cathode are provided to yield a 25 "shorted" cell.

Although the novel features which are believed to be characteristic of this invention will be particularly pointed out in the claims appended hereto, the invention itself, as to its objects and 30 advantages, and the manner in which it may be carried out, may be better understood by referring to the following description, taken in connection with the accompanying drawing forming a part thereof, in which

35 Fig. 1 is a plan view of one type of cell suitable for practicing the invention, and

Fig. 2 is a sectional view of the cell shown in Fig. 1 taken at the line 2—2 thereof.

Referring more particularly to the drawing, 10 40 is a tank of stoneware, or other material which is non-reactive with respect to the stannic chloride electrolyte, provided with a drain or clean-out opening 12 which is closed with a removable plug when the apparatus is in operation.

45 The anode compartment of the cell comprises a permeable diaphragm 14 of canvas or other suitable material supported by a wooden framework 16 within which are zinc plate 18 and zinc rods or strips 20 and zinc scrap 22. If desired 50 plate 18 and rods 20 may be of other conductive material such as graphite so long as care is exercised in seeing that there is good contact between them and the zinc or equivalent anodic metal which is electropositive with respect to tin. The 55 cathode 24 which is of copper or equivalent metal

electronegative to tin is connected with the anode by wires 26 thereby preventing accumulation of precipitated tin on the electropositive metal of the anode. The level of the stannic chloride electrolyte in tank 10 is indicated at 28.

5 In operation the scrap zinc rapidly dissolves and the tin deposits at the cathode 24 from which it falls to the bottom of the tank 10 collecting as a sludge 30 and is removed via the clean-out opening 12. The impurities in the scrap zinc 10 which will not enter into solution in the presence of an excess of zinc are retained within the permeable anode compartment and are thereby prevented from contaminating the precipitated tin. The tin is withdrawn from the tank and 15 appropriately melted down and cast.

The following specific example will serve to illustrate the invention: to 100 volumes of stannic chloride having a specific gravity of 2.28 and analyzing 45.5% (103.7 parts by weight) tin, 20 there were added 140 volumes of water which gave a clear solution of tin tetrachloride. Care was used in adding the water in view of its vigorous reaction with stannic chloride.

The aqueous stannic chloride electrolyte was 25 placed in a cell such as heretofore has been described and illustrated in the drawing. An excess of some 200 parts by weight of zinc scrap was provided in the anode compartment. Solution of the zinc was rapidly effected and the tin 30 deposited at the cathode settled quickly to the bottom of the tank.

The tin sludge was put through a filter press and the filter cake slowly dried. The filtrate (138 volumes) analyzed only 4.8 grams of tin 35 per liter. The dried cake was melted under a sodium chloride-zinc chloride cover slag, the slag removed and the tin metal cast. There was obtained 100 parts by weight metal analyzing over 99% tin which represented a recovery of approximately 97% of the tin in the original stannic chloride.

40 What is claimed is:

1. The process for recovering tin from stannic chloride which comprises adding sufficient water to the stannic chloride to produce an electrolyte therefrom while avoiding production of solid products of hydrolysis, placing the resulting electrolyte into an electrochemical cell including a metal electropositive to tin as an anode and a metal electronegative to tin as the cathode, enclosing the said anode in a permeable diaphragm for retaining solid materials separated from the anode, electrically connecting the anode and 55

cathode to form a shorted cell and allowing the tin to precipitate at the cathode as a sludge.

2. The process for producing tin from stannic chloride which comprises preparing an aqueous 5 solution of the stannic chloride utilizing said solution as the electrolyte in an electrochemical cell having an anode comprising a metal electro-positive to tin and a cathode electronegative to tin electrically connecting the anode and cathode to form a shorted cell, and recovering the precipitated tin.

3. The process for treating secondary metals containing tin which comprises converting the tin to stannic chloride, preparing an aqueous 10 solution of the stannic chloride, utilizing said solution as the electrolyte in an electrochemical cell having an anode comprising zinc and a cathode electronegative to tin electrically connecting the anode and cathode to form a shorted cell, and recovering the tin which deposits from the electrolyte at the cathode.

4. The process for treating secondary metals containing tin which comprises converting the tin to stannic chloride, preparing an aqueous 15 solution of the stannic chloride, utilizing said solution as the electrolyte in an electrochemical cell equipped with an anode comprising a metal which will enter the electrolyte and displace tin therein and a cathode electronegative to tin, said 20 anode and cathode being separated by a permeable diaphragm electrically connecting the anode with the cathode to form a shorted cell, and recovering the tin which is precipitated from the electrolyte by the action of the cell.

35 5. The process for treating secondary metals containing tin which comprises converting the tin to stannic chloride, preparing an aqueous

solution of the stannic chloride, utilizing said solution as the electrolyte in an electrochemical cell equipped with an anode comprising zinc and a cathode electronegative to tin, said anode and cathode being separated by a permeable diaphragm, electrically connecting the anode with the cathode to form a shorted cell, and recovering the tin which is precipitated from the electrolyte by the action of the cell. 5

6. The process for recovering tin from stannic chloride which comprises adding sufficient water to the stannic chloride to produce an electrolyte therefrom while avoiding production of solid products of hydrolysis, placing the resulting electrolyte into an electrochemical cell including a zinc anode and a metal electronegative to tin as the cathode, enclosing the said anode in a permeable diaphragm for retaining solid materials separated from the anode, electrically connecting the anode and cathode to form a shorted 15 cell and allowing the tin to precipitate at the cathode as a sludge. 20

7. The process for recovering tin from stannic chloride which comprises adding sufficient water to the stannic chloride to produce an electrolyte therefrom while avoiding production of solid products of hydrolysis, placing the resulting electrolyte into an electrochemical cell including a zinc anode and a copper cathode, enclosing the said anode in a permeable diaphragm for retaining solid materials separated from the anode, electrically connecting the anode and cathode to form a shorted 25 cell and allowing tin to precipitate at the cathode as a sludge. 30

JESSE O. BETTERTON.  
YURII E. LEBEDEFF.